

06/67

## UNITED STATES PATENT OFFICE

2,135,542

UTILIZATION OF COLLIERY SHALE AND  
OTHER WASTE BITUMINOUS SHALES IN  
THE MANUFACTURE OF CEMENTITIOUS  
PRODUCTS

Norman Victor Sydney Knibbs, Westwood, New Barn, Longfield, and Alfred Petter Pehrson, Streatham, London, England, assignors to The Continental Investment Syndicate Limited, London, England

No Drawing. Application April 3, 1936, Serial No. 72,591. In Great Britain August 8, 1935

3 Claims. (Cl. 18—47.5)

This invention relates to moulded building blocks, artificial stone, paving slabs, moulded pipes and posts and like products which are produced by moulding or otherwise shaping cementitious materials derived from admixtures of lime and argillaceous and/or siliceous materials.

In the mining of coal there is generally produced a considerable quantity of shale or other argillaceous substance which ordinarily is valueless and is discarded, forming the dumps that are to be seen at nearly all collieries. In some few instances this shale has been found suitable for brick-making by the usual process and some other minor uses have been found for small quantities of it, but ordinarily it is valueless and is an expense to dump. Furthermore, because of the combustible it contains the heaps of shale generally take fire and slowly burn, with attendant disadvantages of smoke nuisance, etcetera. In the same way, a low grade oil shale—too poor to use in the retorts—is sometimes produced when mining oil shales of higher quality.

By experiment we have found that the colliery or oil shales are often suitable for making blocks of high quality by the processes described in our pending application Serial No. 62,298, for not only do these shales ordinarily contain sufficient combustible material to calcine themselves and to produce from limestone, chalk or other form of calcium carbonate, the lime required for our processes, but they also ordinarily contain sufficient sulphur in the form of pyrites or otherwise, to produce in burning with limestone sufficient calcium sulphate to enable the special advantages of steam-hardening according to our processes to be obtained or at any rate to contribute materially to this result.

According to the present invention, a moulded or otherwise formed article is made by steam-hardening under pressure a cementitious material produced in the known manner by calcining the shale with limestone, chalk or other form of calcium carbonate, the combustible of the shale at least contributing to that necessary for effecting calcination of the shale-lime mixture, crushing and/or grinding the mixture, and adding water. With previously proposed processes the wet mass was merely moulded or otherwise formed into the required article without being subjected to steam-hardening.

The steam-hardening of the shale-lime mixture which characterizes the present invention is preferably performed in autoclaves at a pressure of about 120 lbs. per square inch.

We have found that when a cementitious ma-

terial such as that above mentioned is subjected to the action of steam under pressure, any deleterious sulphides—that is to say sulphides liable to oxidize and cause expansion on subsequent exposure—are hydrolyzed and the sulphur evolved as hydrogen sulphide. The steam-hardening process therefore turns a faulty material into a sound one. It will be appreciated that where the term "shale" is used in the following description, it is intended to imply colliery shale or other argillaceous wastes from mining coal, bituminous shale, low grade oil shale, and similar combustible containing waste argillaceous or siliceous products.

Although it is preferred that the shale used in the production of the cementitious material should contain combustible sufficient to effect calcination not only of itself but also of the calcium carbonate of the shale-lime mixture, we wish it to be understood that the invention also extends to cases in which coal or other fuel is added to supplement the combustible matter in the shale. In the following description, which may be said to be a preferred embodiment, it will be assumed that the combustible of the selected shale effects calcination of the shale-lime mixture. Moreover, although limestone may generally be the most convenient form of calcium carbonate, any other form of calcium carbonate which may be available can be used.

The proportion of shale to limestone that is used will depend upon the amount of combustible matter in the shale and upon the use to which the mixture is put. We have found that some shales we have tried will calcine about their own weight of limestone in addition to themselves, while others will not calcine nearly as much limestone. A suitable plant for the calcination of the mixture is a short shaft kiln, similar to a short lime kiln, and the height required will vary with the size of the shale and limestone used. We have found that ordinarily it is preferable but not essential to have the shale and limestone of roughly the same size.

For crushing and grinding the mixture any suitable machines may be used, such as a jaw-crusher, followed by a tube mill. Hydration if required may be carried out by known methods.

The ground mixture contains silica and alumina, combined or free, and free lime, and it is therefore a potential source of calcium silicates and aluminates. The ground mixture after mixing with water and after the lime has hydrated will harden to produce a mass of high

strength when it is subjected to the action of steam under pressure.

To effect hydration of the lime, if required, water is added equivalent to between 33% and 5 45% of the weight of lime in the mixture, which is then put into bunkers and left to stand till hydration has been completed whereafter further water is added to the mass which is then passed to the moulds or like shaping devices.

10 For use in steam-hardened blocks or other articles, the mixture may be ground to a fineness of 95% passing a sieve of 100 meshes to the linear inch. Generally, the optimum lime content is about 20 to 25 per cent. by weight of 15 the calcined mixture and the shale and limestone are therefore mixed in a proportion to produce this calcined mixture.

The mixture after grinding and with or without hydration of the lime may be used instead of 20 Portland or other cement to produce building blocks, moulded or otherwise formed articles such as posts, pipes, asbestos-cement sheets, et cetera, decorative mouldings, et cetera, the moulded or formed articles being finished by 25 steam hardening. The mixture may be used instead of lime in sand-lime bricks, in which case the mixture ordinarily is ground to a lesser degree of fineness than that previously mentioned. Aluminium dust or other gas-generating agent 30 may be added to the mixture to produce porous blocks and like articles.

In the production of building blocks and like moulded articles according to the present invention, it is preferable that the general processes 35 as described in our pending application, Serial No. 62,298, should be used. It may be observed that this application deals with the effects of an inclusion with the mixture of a compound of an oxy-acid of sulphur, and in this connection it 40 may be mentioned that colliery shale and like materials ordinarily contain sulphides which on calcination produce sulphur oxides, but if the shale is calcined by itself a greater part of the

oxide compounds is lost, and it is only when the mixture is calcined that the oxides are absorbed by the lime and thus retained to form calcium sulphate.

For asbestos-cement products the requisite 5 quantity of asbestos can be added to the mixture while in a similar way, sand gravel, crushed stone or other aggregate or mixtures of aggregates may be added.

What we claim then is:—

1. A method of making a cementitious product that comprises mixing fuel-containing shale with calcium carbonate, utilizing the fuel contained in the shale to at least partly calcine the shale and the calcium carbonate to produce 15 quicklime, dividing the calcined mixture into smaller parts, adding water, shaping to the required form, hydrating the quicklime, and applying steam under pressure to harden.

2. A method of making a cementitious product 20 that comprises mixing fuel-containing and sulphur-containing shale with calcium carbonate, utilizing the fuel contained in the shale to at least partly calcine the shale and the calcium carbonate to produce quicklime and to produce 25 calcium sulphate by the reaction of the sulphur with the calcium carbonate, dividing the calcined mixture into smaller parts, adding water, shaping to the required form, hydrating the quicklime, and applying steam under pressure to 30 harden.

3. A method of making a cementitious product that comprises mixing fuel-containing shale with calcium carbonate, utilizing the fuel contained in the shale to at least partly calcine the shale 35 and the calcium carbonate to produce quicklime, adding a gas-generating agent to the mass to render it cellular, dividing the calcined mixture into smaller parts, adding water, shaping to the required form, hydrating the quicklime, and applying steam under pressure to harden.

NORMAN VICTOR SYDNEY KNIBBS.

ALFRED PETTER PEHRSON.